

# UNITED STATES PATENT OFFICE.

MARK JOHN MASTERS, OF NEW YORK, N. Y., ASSIGNOR OF THREE FOURTHS  
TO BASIL D. VASSILIADES, CONSTANTINE D. VASSILIADES, AND ALEX-  
ANDER D. VASSILIADES, ALL OF SAME PLACE.

## ADHESIVE POWDER FOR GILDING, &c.

SPECIFICATION forming part of Letters Patent No. 388,984, dated September 4, 1888.

Application filed November 1, 1887. Serial No. 254,017. (No specimens.)

*To all whom it may concern:*

Be it known that I, MARK JOHN MASTERS, of the city, county, and State of New York, have invented a new and useful Improvement 5 in Adhesive Powders for Metal Stamping on Fabrics, &c., of which the following is a specification.

My invention relates to a new powder, whereby I am enabled to cause gold, silver, 10 or other metal leaf to adhere to the surface of silk, card-board, paper, leather, satin, cloth, celluloid, ivory, wood, veneers, or any other material upon which stamped designs in metal are desired.

15 I prepare my said powder in the following manner: Equal parts of gum-sandarac and best golden yellow shellac are melted together in a water-bath, and there boiled for a period of about five hours. The mixture is constantly 20 stirred, so as to insure thorough mingling of the ingredients. At the end of the above time the compound is poured out upon a greased flat slab, so as to form a sheet about one-quarter inch in thickness, which is allowed to cool 25 and harden. After hardening, said sheet is broken up and ground to a very fine powder.

I use this powder for the purpose named by applying it in a fine dust upon the surface to be stamped. Upon the powder thus applied

I place a leaf of the desired metal, and then 30 subject said leaf to the pressure of a suitably-formed die, heated to a point sufficient to cause fusion of the said powder beneath the leaf. In this way the leaf is caused to adhere to the material at all points covered by the 35 design. The loose powder and leaf outside the edges of the design are finally brushed off.

I find that by means of this powder I can stamp designs in metal upon materials of the smoothest surface—such as highly-finished 40 ivory, celluloid, or pasteboard—with remarkable sharpness and luster.

In other applications for Letters Patent simultaneously herewith filed by me I have fully described and claimed the process of 45 manufacture of the aforesaid powder, and also the process of stamping in metal leaf by the aid thereof. The subject-matter of said applications is therefore herein disclaimed.

I claim—  
50 The powder composed of gum-sandarac and shellac, as and for the purpose set forth.

MARK JOHN MASTERS.

Witnesses:

PARK BENJAMIN,  
EDGAR GOODWIN.